

## UNITED STATES PATENT OFFICE

2,252,399

## SURFACE COVERING MATERIAL

Walter W. Durant, Old Greenwich, Conn., assignor to American Cyanamid Company, New York, N. Y., a corporation of Maine

No Drawing. Application November 30, 1939,  
Serial No. 306,902

3 Claims. (Cl. 106—264)

This invention relates to the improvement in the alkali resistance of surface covering compositions such as floor covering compositions containing siccative binders.

An object of this invention is to improve the alkali resistance of surface covering compositions containing siccative binders.

This and other objects are attained by incorporating in a siccative composition which is to be used in a floor covering composition or other surface covering composition a nitrile, containing at least one carbon-carbon double bond, preferably one containing a terminal carbon-carbon unsaturation.

The following example is given by way of illustration and not in limitation.

## Example

|               | Parts by weight |
|---------------|-----------------|
| Binder        | 30              |
| Wood flour    | 30              |
| Whiting       | 20              |
| Lithopone     | 20              |
| Acrylonitrile | 3               |

These substances with or without a small proportion of drier, e. g. 0.1% cobalt naphthenate, are mixed together, e. g. in an internal mixer. The compacted mass which is delivered from the mixer may be disintegrated, as by a set of "scratch rolls" which comprises a plurality of rolls having intermeshing teeth projecting from their surfaces. The resulting material is sheeted on calender rolls or optionally it may be further mixed and disintegrated and then calendered. The material may be calendered on to burlap or other fibrous backing if desired. The sheeted material is placed in a stoving oven through which a current of heated air from about 70° C. to about 90° C. is circulated until the material is completely "seasoned," i. e. until the sheet acquires the necessary degree of hardness.

The hardness may be measured by any of the methods generally employed in the manufacture of linoleum. See the Federal Stock Catalogue (U. S. Government Printing Office), section 4, part 5, pages LLL-L-351 et seq. and pages LLL-L-361 et seq., for the method employed herein. The time required for "seasoning" a 2 mm. sheet of the above composition is about twelve days. The resulting "seasoned" floor covering shows improved alkali resistance. One method of determining alkali resistance is to measure the depth in millimeters to which a 5% solution of sodium hydroxide in water penetrates in one hour at a temperature of 70° F. By this method

the alkali resistance of the "seasoned sheets" is about 0.17 mm. penetration.

The "seasoning speed" of a 2 mm. sheet of the same mixture which does not contain acrylonitrile is about twelve to fourteen days and the alkali resistance of such a composition is about 0.28 mm. The marked improvement obtained with my composition is outstanding inasmuch as I have found it to be very difficult to improve the alkali resistance by even as little as 0.01 mm.

The binders may be derived from the drying oils and may be made in any convenient well-known manner, such as the methods described in British Patent 305,656 or the binders may comprise any of the various alkyd resins having siccative properties. For drying oil binders, linseed oil is preferable for economic reasons but other siccative oils may be used such as, for example, menhaden or fish oil, tung oil, soy bean oil, perilla oil, otticica oil, Scheiber oil, sunflower seed oil, etc. The term "siccative oil" as used herein is intended to include not only the so-called drying oils but also the so-called semi-drying oils. Furthermore it is possible to use mixtures of siccative oils with other fatty oils of the non-drying type.

It may be preferable in the manufacture of linoleum to make use of so-called "scrim-oil" or "shed oil" either alone or fluxed with rosin or other gums or resins and/or mixed with a proportion of the so-called "mechanical oil." Either of these types of oils may be used singly if desired.

In the preparation of the siccative oil binders it is customary to use rosin in admixture with the oil although other substances of the same type may be used, e. g., kauri gum, Congo gum, ester gum, abietic acid and its esters, pimaric acid, etc.

Other siccative binders which may be used are the alkyd resins which have siccative properties. Among these, the drying oil modified reaction products of maleic or fumaric acid with terpenes and polyhydric alcohols are particularly desirable. Other alkyd resins which are modified with drying oils may be used such as the phthalic-glyceride resins, the glycol-maleic resins, and mixed resins such as the phthalic-fumaric-glycol-glyceride resins.

Instead of wood flour and/or the whiting and lithopone used in the examples, other fillers or pigments may be used. Examples of such fillers are: cork, cellulose pulp, asbestos, cottonwood tree pulp, walnut shell meal, glass fibers, foliated glass, etc. Among the pigments which may be

used the following are included: lithopone, bar-  
rytes, zinc oxide, titanium oxide, chromates, red  
lead, white lead, malachite green, chrome green,  
chrome yellow, Prussian blue, iron oxide, etc.  
Similarly dyes and lakes may be used if de-  
sirable.

It is generally preferable to use driers in the  
preparation of the binders. The drier is usually  
added to the binder during the oxidation process  
and if desirable additional drier may be added  
when the binder, fillers, etc., are mixed together.  
Suitable driers include the oil soluble salts such  
as the naphthenates, resinates and linoleates of  
cobalt, lead, manganese, zinc, and chromium.  
Only a small proportion of these driers based on  
the siccative oil content, is generally sufficient,  
e. g. about 0.005-1%, although larger proportions  
may be used as expedient. Obviously various  
mixtures of driers may be used.

The term "seasoning" as applied to linoleum  
compositions indicates the process of curing by  
heating or equivalent treatment to polymerize  
and/or oxidize the composition to a stage where-  
in the floor covering is sufficiently hard and  
resistant to abrasion to be suitable for its in-  
tended purpose and yet is still sufficiently flexi-  
ble to permit the usual bending and rolling re-  
quired of linoleum. The term "maturing" is  
similarly used.

Other unsaturated nitriles may be used to im-  
prove the alkali resistance of surface covering  
compositions, e. g. substituted acrylonitriles  
(such as methacrylonitrile and ethacrylonitrile),  
4-butene-1-nitrile, the pentene-nitriles, etc.

I have found that only a small proportion of

the nitriles is generally sufficient, e. g. 0.1-5%  
of the siccative composition but obviously smaller  
or larger proportions may be used if desirable.

The nitrile may be added during the mixing  
of the binder with the fillers, etc., or it may be  
added before or during the oxidation of the  
binder.

Obviously many modifications in the processes  
and compositions described above may be made  
without departing from the spirit and scope of  
the invention as defined in the appended claims.

I claim:

1. In a process of curing a surface covering  
composition including a siccative material se-  
lected from the group consisting of drying oils  
and drying oil modified polyhydric alcohol-poly-  
carboxylic acid resins, the step which comprises  
adding to such a composition an unsaturated ni-  
trile.
2. In a process of curing a surface covering  
composition including a siccative material se-  
lected from the group consisting of drying oils  
and drying oil modified polyhydric alcohol-poly-  
carboxylic acid resins, the step which comprises  
adding to such a composition an unsaturated ni-  
trile having a terminal carbon-carbon double  
bond.
3. In a process of curing a surface covering  
composition including a siccative material se-  
lected from the group consisting of drying oils  
and drying oil modified polyhydric alcohol-poly-  
carboxylic acid resins, the step which comprises  
adding to such a composition acrylonitrile.

WALTER W. DURANT.